

# United States Patent [19]

Kumagae et al.

[11] Patent Number: 4,466,902

[45] Date of Patent: Aug. 21, 1984

## [54] RUST INHIBITOR

[75] Inventors: Shinichi Kumagae, Toyonaka; Tatsuo Manabe, Osaka, both of Japan

[73] Assignee: Ipposha Oil Industries, Co., Ltd., Osaka, Japan

[21] Appl. No.: 428,719

[22] Filed: Sep. 30, 1982

## [30] Foreign Application Priority Data

Jan. 31, 1982 [JP] Japan ..... 57-13527  
May 19, 1982 [JP] Japan ..... 57-85256

[51] Int. Cl.<sup>3</sup> ..... C23F 11/19; C23F 11/12;  
C23F 11/16

[52] U.S. Cl. ..... 252/391; 252/393;  
252/397; 252/404; 252/407; 564/156;  
106/14.13

[58] Field of Search ..... 252/393, 397, 404, 407,  
252/391; 564/156; 106/14.13

## [56] References Cited

### U.S. PATENT DOCUMENTS

4,105,629 8/1978 Minagawa et al. ..... 252/404  
4,263,167 4/1981 Mago ..... 252/393  
4,364,846 12/1982 Kaufman ..... 252/393

### OTHER PUBLICATIONS

Chemical Abstracts, 74, 112472q, 1971.

Lenk, *Journal of Applied Polymer Science*, vol. 15, pp.  
311-315, (1971).

Chemical Abstracts 53, 19378 gh, 1959.

Chemical Abstracts 94, 161207 d.

Primary Examiner—Richard D. Lovering

Assistant Examiner—Anne Brookes

Attorney, Agent, or Firm—Armstrong, Nikaido,  
Marmelstein & Kubovcik

[57]

## ABSTRACT

A rust inhibitor comprising, as an effective component, at least one compound having the following general formulae (A), (B) and (C)



and



wherein  $\text{R}_1$  and  $\text{R}_2$  are independently a hydrocarbon group having 1 to 6 carbon atoms,  $\text{R}_3$  and  $\text{R}_4$  are independently a hydrocarbon group having 1 to 4 carbon atoms or a hydrocarbon group containing an aromatic ring and having 6 to 12 carbon atoms,  $\text{R}_5$  and  $\text{R}_6$  are independently a hydrocarbon group having 1 to 18 carbon atoms,  $m$  and  $n$  are independently 0 or an integer of 1 to 3,  $\text{R}_3$  or  $\text{R}_4$  is hydrogen in the case of  $m$  or  $n$  is 0,  $\text{X}$  is O, S,  $\text{SO}_2$ , CO or a hydrocarbon group having 1 to 9 carbon atoms,  $Y$  is an aromatic hydrocarbon group having 6 to 10 carbon atoms, and  $M$  is a cation. This rust inhibitor has an excellent rust preventing effect for a wide variety of metals, a good stability against chemicals and oxidation and a low toxicity and is easily applicable in either a water-soluble state or an oil-soluble state.

9 Claims, No Drawings

## RUST INHIBITOR

The present invention relates to a novel water-soluble and/or oil-soluble rust inhibitor. More specifically, it relates to a carboxylate type rust inhibitor having an excellent rust preventing capability for a wide variety of metals, a low toxicity and good stability, and which is easily applicable to a wide variety of metals in either a water-soluble or an oil-soluble state.

Various kinds of rust inhibitors have been heretofore developed in various application fields. However, a rust inhibitor having an excellent rust preventing capability for a wide variety of metals, a low toxicity, good stability and easy applicability has not been substantially developed.

For instance, oil-soluble type rust inhibitors such as petroleum sulfonates, alkylaryl sulfonates, oxidized waxes, sorbitan fatty acid esters, metallic soaps and other various agents have been used as a relatively long-term rust inhibitor. However, these oil-soluble type rust inhibitors involve a problem in that the removal thereof is relatively difficult when the applied rust inhibitors should be removed at a later step. Furthermore, oil-soluble type rust inhibitors involve a problem from the viewpoint of flammability, the working atmosphere and the effective usage of resources. Thus, there has been a tendency in the art that aqueous type rust inhibitors are desired. In order to solve the above-mentioned problems, an attempt has been made to use oil-soluble type rust inhibitors in the form of emulsion by dispersing or emulsifying the same in water. However, rust inhibitors having a satisfactory rust preventing effect have not been developed due to, for example, the drawbacks of emulsifying agents.

Furthermore, water-soluble compounds having an excellent rust preventing effect, for example, inorganic salts, such as, chromates, phosphates and nitrites are known in the art. However, the use of these inorganic salts has been limited from the viewpoint of pollution control, because chromates have strong toxicity, phosphates result in eutrophic waste water and nitrites, together with a lower amine, form nitrosamine, which seems to be a carcinogen.

Known water-soluble or oil-soluble organic rust inhibitors include various organic compounds such as alkyl amines, alkyl polyamines, alkylol amines, benzotriazoles, alkyl phosphate type surfactants, long-chain alkyl quaternary ammonium salts, alkyl imidazolinium salts, salts of alkylated benzoic acid and addition products of alkylene oxides and amines. These organic rust inhibitors are generally used, in combination with inorganic rust preventing salts such as sodium nitrite, because the rust preventing effect of the above-mentioned known organic rust inhibitors is not satisfactory. However, the combined use of the water-soluble organic rust inhibitor with the inorganic rust inhibitors involves a problem that the compatibility thereof is not sufficient, the stability of the rust preventing preparation containing both inhibitors is not satisfactory and the desirable rust preventing effect is lost when the rust inhibitors are continuously used. In addition, many organic rust inhibitors have surface activity and, therefore, tend to cause foaming when they are used in an aqueous medium. The foaming is a problem in a rust preventing treatment because the workability and the rust preventing effect are decreased.

Furthermore, rust preventing treatments are applied to various substances including steel and various other metals. Recently, a plurality of metals have been often subjected to simultaneous rust preventing treatments. Thus, a rust inhibitor capable of simultaneously preventing the generation of rust on many kinds of metals is often desired in the art.

The objects of the present invention are to eliminate the above-mentioned problems of the prior art and to provide an organic rust inhibitor which has an excellent rust preventing effect on steel and other metals in a small amount, without using an inorganic compound together, and which can be advantageously used, together with various conventional rust inhibitors, to exhibit an excellent rust preventing effect on steel and a plurality of various other metals.

Another object of the present invention is to provide an organic rust inhibitor having an excellent chemical stability and anit-oxidation property, a good mechanical lubricity and a low foaming property.

Other objects and advantages of the present invention will be apparent from the description set forth hereinbelow.

In accordance with the present invention, there is provided a rust inhibitor comprising, as an effective component, at least one compound having the following general formulae (A), (B) and (C):



wherein R<sub>1</sub> and R<sub>2</sub> are independently a hydrocarbon group having 1 to 6 carbon atoms, R<sub>3</sub> and R<sub>4</sub> are independently a hydrocarbon group having 1 to 4 carbon atoms or a hydrocarbon group containing aromatic ring and having 6 to 12 carbon atoms, R<sub>5</sub> and R<sub>6</sub> are independently a hydrocarbon group having 1 to 18 carbon atoms, m and n are independently 0 or an integer of 1 to 3, R<sub>3</sub> or R<sub>4</sub> is hydrogen in the case of m or n is 0, X is O, S, SO<sub>2</sub>, CO or a hydrocarbon group having 1 to 9 carbon atoms, Y is an aromatic hydrocarbon group having 6 to 10 carbon atoms and M is a cation. The hydrocarbon groups R<sub>1</sub>, R<sub>2</sub>, R<sub>3</sub>, R<sub>4</sub>, R<sub>5</sub> and R<sub>6</sub> in the above-mentioned formulae (A), (B) and (C) may be linear or branched hydrocarbons and may contain an unsaturated bond or bonds.

Examples of the dicarboxylic acids of the dicarboxylic acid salts of the above-mentioned formulae (A), (B) and (C) are: bis(4-oxyphenyl)sulfide-o,o-dialkylcarboxylic acids such as bis(4-oxyphenyl)sulfide-o,o-dipropionic acid; bis(4-oxyphenyl)sulfone-o,o-dialkylcarboxylic acids such as bis(4-oxyphenyl)sulfone-o,o-diacetic acid and bis(4-oxyphenyl)sulfone-o,o-dipropionic acid; bis(4-oxyphenyl) ketone-o,o-dialkylcarboxylic

acids such as bis(4-oxyphenyl) ketone-o,o-diacetic acid; bis(4-oxyphenyl)alkane-o,o-dialkylcarboxylic acids such as bis(4-oxyphenyl)methane-o,o-diacetic acid,  $\beta,\beta$ -bis(4-oxyphenyl)propane-o,o-diacetic acid,  $\beta,\beta$ -bis(4-oxyphenyl)propane-o,o-dipropionic acid and bis(4-oxyphenyl)methane-o,o-dibutyric acid; 2,2'-methylenebis(4-ethyl-6-tert-butylphenoxyacetic acid); 2,2'-methylenebis(4-methyl-6-tert-butylphenoxypropionic acid); bis[(benzyl)-4-oxyphenyl]alkane-o,o-dialkylcarboxylic acids such as bis[(benzyl)-4-oxyphenyl]methane-o,o-diacetic acid; bis(4-oxycyclohexyl)alkane-o,o-dialkylcarboxylic acids such as bis(4-oxycyclohexyl)ethane-o,o-dipropionic acid; N,N'-terephthaloyldiglycine, N,N'-terephthaloyldiaminopropionic acid, N,N'-terephthaloyldiaminocaproic acid, N,N'-terephthaloyldialanine, and N,N'-terephthaloyldisarcosine.

These dicarboxylic acids may be produced by any conventional method. For instance, the dicarboxylic acids corresponding to the compounds having the above-mentioned general formula (A) can be readily produced from the corresponding diphenol compounds and halogeno carboxylic acids. The dicarboxylic acids corresponding to the compounds having the above-mentioned general formula (B) can be produced either by hydrogenating the above-mentioned dicarboxylic acids corresponding to the compounds having the general formula (A) or by reacting dicyclohexanol compounds with halogeno carboxylic acids. Furthermore, the dicarboxylic acids corresponding to the compounds having the above-mentioned general formula (C) can be readily produced by reacting o-, m- and p-phthaloyl chlorides and amino acids.

Examples of the cations in the above-mentioned general formulae (A), (B) and (C) are those derived from the reactions of the above-mentioned dicarboxylic acids and alkaline (or basic) compounds. The alkaline compounds usable in these reactions are: alkali metal salts such as sodium hydroxide, potassium hydroxide, sodium carbonate, sodium phosphate, and potassium phosphate; alkaline earth metal salts such as calcium hydroxide, and barium hydroxide; ammonia, amines such as methylamine, ethylamine, isopropylamine, trimethylamine, monoethanolamine, diethanolamine, triethanolamine, isopropanolamine, aminomethyl methanol, cyclohexylamine, and morpholine. Furthermore, various metal salts and alkylamines, other than the above-exemplified compounds, can also be used in the preparation of the above-mentioned compounds (A), (B) and (C).

The above-mentioned compounds (A), (B) and (C) can be produced by mixing the corresponding dicarboxylic acids and the alkaline compounds in a reaction solvent. The reaction mixture can optionally be heated. Any solvent which is capable of dissolving or dispersing both the components can be advantageously used. Examples of such solvents are water, organic solvents such as methanol, ethanol and methyl ethyl ketone and oils such as spindle oil and machine oil and any mixture thereof.

The dicarboxylic acids and the alkali compounds can be mixed in an equivalent amount or in a small excess of an either component. Generally speaking, the use of an excess amount of the alkaline compounds results in water-soluble rust inhibitors, whereas the use of an excess amount of the dicarboxylic acids results in oil-soluble rust inhibitors.

The rust inhibitors of the present invention can be advantageously used in the form of a solution, or a

dispersion in water or oil, or in the form of an emulsion, as in the conventional rust inhibitors.

In order to use as a water-soluble type rust inhibitor, the above-mentioned compounds (A) and (B) in which R<sub>3</sub> and R<sub>4</sub> are hydrocarbon groups with a relatively small number of carbon atoms and m and n are zero or a small integer and which are produced by using an alkali metal salt, ammonia, a lower amine or a lower alkylolamine are desired. Contrary to this, in order to use as an oil-soluble type rust inhibitor, the above-mentioned compounds (A) and (B), in which R<sub>3</sub> and R<sub>4</sub> are hydrocarbon groups with a relatively large number of carbon atoms or including an aromatic ring and m and n are a relatively large integer (e.g., 2 or 3) and which are produced by using an alkaline earth metal salt or an amine having a relatively large molecular weight.

The above-mentioned dicarboxylic acid salt type compounds (A), (B) and (C) have an excellently high thermal stability and anti-oxidation stability since they contain as a basic skeleton an aromatic or alicyclic ring therein. Thus, the rust inhibitor of the present invention can be advantageously used as an effective component of a rust preventing preparation and also as a rust preventing additive for a lubricating oil, a machining oil, and a grinding oil.

Furthermore, the above-mentioned compounds (A), (B) and (C) have a lipophilic group in the center of the structure and hydrophilic groups on both sides of the lipophilic group. This specific chemical structure of the above-mentioned compounds result in an excellent orientation of the compounds on a metallic surface to be applied. Furthermore, the foaming power of the above-mentioned compounds (A), (B) and (C) is very poor, so that the present rust inhibitor has no substantial problem often caused by the foaming during a conventional rust preventing treatment and has an excellent workability.

Thus, the rust inhibitor according to the present invention has an extremely excellent rust preventing effect and exhibit a sufficient rust prevention in a small amount even without using another inorganic or organic rust inhibitor. Especially, as illustrated in Examples hereinbelow, the present rust inhibitor exhibited effective and wide range rust preventing properties both in a wet cast iron powder test and a rust preventing test of iron plates in a humidity cabinet according to a Japanese Industrial Standard (JIS) method. Most of the conventional rust inhibitors does not exhibit effective rust prevention in these tests.

The present rust inhibitor has an excellent chemical stability, anti-oxidation properties and low foaming properties, in addition to the above-mentioned excellent rust preventing effects, and, therefore, the present rust inhibitor can also be widely used, as a rust preventing additive in, for example, the following various compositions:

- (1) A water-soluble rust preventing preparation for steel free from sodium nitrite;
- (2) A water-soluble rust preventing preparation for various metals, used together with other water-soluble inorganic or organic rust inhibitors;
- (3) A coolant;
- (4) A lubricant;
- (5) A water-soluble type cutting and grinding preparation;
- (6) An emulsion type cutting and grinding preparation;
- (7) A lubricating oil, a cutting oil, a grinding oil, a metal working oil, a milling or rolling oil, a draw-

ing oil, a wire drawing oil, a punching oil, and an extrusion processing oil;

- (8) A coating composition; and  
(9) A detergent composition.

The present invention will now be further illustrated by, but is by no means limited to, the following Examples, wherein all parts and percentages are expressed on a weight basis unless otherwise noted.

#### EXAMPLE 1

Two hundred and fifty parts of bis(4-oxyphenyl)sulfone, 96 parts of sodium hydroxide and 800 parts of water were charged into a reactor provided with a condenser and a stirrer. The mixture was dissolved upon heating.

When the temperature of the reactor content became 90° C. to 95° C., a mixed solution of 257 parts of sodium monochloroacetate and 500 parts of water was dropwise added to the reactor for 30 to 60 minutes while stirring and, then, the reaction mixture was allowed to react for 3 hours at the same temperature while stirring.

After cooling, the reaction mixture was acidified by sulfuric acid to precipitate the resultant dicarboxylic acid in the reaction mixture. The precipitated dicarboxylic acid was filtered and, then, washed with water. Thus, bis(4-oxyphenyl)sulfone-o,o-diacetic acid in the form of white powder was obtained.

Then, 100 parts of bis(4-oxyphenyl)sulfone-o,o-diacetic acid, 78 parts of triethanolamine and 415 parts of water were mixed under heating. Thus, a rust preventing composition containing, as an effective component, 30% of the triethanolamine salt of bis(4-oxyphenyl)sulfone-o,o-diacetic acid was prepared.

#### EXAMPLE 2

Two hundred and twenty-eight parts of  $\beta,\beta$ -bis(4-oxyphenyl)propane, 280 parts of sodium monochloroacetate, 200 parts of methanol and 300 parts of water were charged into the same reactor as used in Example 1 and the mixture was heated to a temperature of 80° C. to 85° C. while stirring to form a clear solution. A mixed solution of 105 parts of sodium hydroxide and 200 parts of water was dropwise added to the reactor for 30 to 60 minutes at the same temperature while stirring and, then, the mixture was allowed to react for 3 hours at the same temperature while stirring.

After cooling, the reaction mixture was acidified with sulfuric acid to precipitate the resultant dicarboxylic acid, followed by filtration and water washing. Thus, 317 parts of  $\beta,\beta$ -bis(4-oxyphenyl)propane-o,o-diacetic acid in the form of white powder was obtained.

The resultant  $\beta,\beta$ -bis(4-oxyphenyl)propane-o,o-diacetic acid was converted into the triethanolamine salt and a rust preventing composition containing 30% of the effective component was prepared in the same manner as in Example 1.

#### EXAMPLE 3

Bis(4-oxyphenyl)methane-o,o-dipropionic acid was obtained from 198 parts of bis(4-oxyphenyl)methane, 192 parts of sodium hydroxide, 980 parts of water and 220 parts of monochloropropionic acid in the same manner as in Example 1. The resultant bis(4-oxyphenyl)-o,o-dipropionic acid was neutralized with triethanolamine in a manner as described in Example 1 to convert it into the triethanolamine salt and a rust preventing composition containing 30% of the effective

component was prepared in the same manner as in Example 1.

Various salts of bis(4-oxyphenyl)-o,o-dipropionic acid listed in Table 3 below were prepared in the same manner as in Example 1 and rust preventing compositions containing 30% of the effective components were prepared from the resultant salts.

#### EXAMPLE 4

10 Triethanolamine salt of 2,2'-methylenebis(4-ethyl-6-tert-butylphenoxyacetic acid) was prepared from 2,2'-methylenebis(4-ethyl-6-tert-butyl phenol) and sodium monochloroacetate in the same manner as in Example 1. The results are shown in Table 3.

#### EXAMPLE 5

20  $\beta,\beta$ -Bis[(benzyl)-4-oxyphenyl]propane-o,o-diacetic acid was prepared from  $\beta,\beta$ -bis[(benzyl)-4-oxyphenyl]-propane and sodium monochloroacetate and was converted into the triethanolamine salt in the same manner as in Example 1. A rust preventing composition containing 30% of the effective component was prepared in the same manner as in Example 1.

#### EXAMPLE 6

25 Bis(4-cyclohexyl)ethane-o,o-dipropionic acid was prepared from bis(4-oxycyclohexyl)ethane and monochloropropionic acid and was converted into the triethanolamine salt in the same manner as in Example 3. A rust preventing composition containing 30% of the effective component was prepared in the same manner as in Example 3.

#### EXAMPLE 7

30 One hundred parts of 2,2'-methylenebis(4-ethyl-6-tert-butylphenoxyacetic acid obtained in Example 4 was mixed with 16 parts of calcium hydroxide (an equivalent ratio was 1:1.05) and the mixture was heated to a temperature of 150° C. to 160° C. for 3 hours while stirring. The resultant mixture was cooled to a temperature of 110° C. and, then, 2185 parts of a spindle oil was added to the mixture. After allowing the mixture to cool, the unreacted calcium was removed from the mixture by decantation to obtain an oil-soluble type rust preventing composition containing 5% of the calcium salt.

35 Oil-soluble type rust preventing compositions containing the magnesium salt and the barium salts were also prepared in the same manner as in the calcium salt.

40 These oil-soluble type rust preventing compositions were diluted twice by the spindle oil and kerosine prior to the evaluation of the rust preventing compositions set forth hereinbelow.

#### Comparative Example 1

45 One hundred parts of benzoic acid, 117 parts of triethanolamine and 506 parts of water were stirred under heating. Thus, an aqueous composition containing 30% of the triethanolamine salt of benzoic acid was obtained.

50 This is a sample of a conventional water-soluble type rust inhibitor component.

#### Comparative Example 2

55 One hundred parts of oleic acid, 51 parts of triethanol and 352 parts of water were stirred under heating. Thus, a rust preventing composition containing 30% of the triethanolamine salt of oleic acid was obtained.

## Comparative Example 3

One hundred parts of sebacic acid, 160 parts of triethanolamine and 615 parts of water were mixed while stirring to prepare a rust inhibitor composition containing about 30% of the effective component. This is a sample of a conventional water-soluble type rust preventing composition having a characteristic low foaming property.

## Comparative Example 4

Thirty parts of the triethanolamine salt of oleylsarcosine, 30 parts of butylcellosolve and 40 parts of water were mixed to prepare a water-soluble type rust preventing composition.

## Comparative Example 5

Twenty parts of the triethanolamine salt of alkylphosphoric acid ester, 3 parts of sodium benzoate, 7 parts of sodium nitrite and 70 parts of water were mixed to prepare a water-soluble type rust preventing composition in which an organic compound was used in combination with an inorganic compound.

The rust preventing compositions prepared in Examples 1 to 7 and Comparative Examples 1 to 5 were evaluated by the following test methods. The results are shown in Tables 1 to 4 below.

## &lt;Test Methods&gt;

## (1) Evaluation test of rust preventing property under humidity conditions

The evaluation was carried out according to a JIS-K-2246 method. SPCC-1 steel test panels were dipped in a test composition (i.e., 1% aqueous solutions of the water-soluble rust inhibitors or oil-soluble rust inhibitor compositions having the given concentration) and was, then, air dried. The rusting of the steel panels was tested in a humidity cabinet under the conditions of a temperature of  $49 \pm 1^\circ \text{C}$ , R.H. (relative humidity) of more than 95% and an air feed amount of  $886.5 \pm 110.5$  liter/hour.

The evaluation of the rust generation was made according to a JIS-K-2246 method and based on the following classification.

- A: No rusting
- B: Less than 10% rusting generation
- C: Less than 25% rusting
- D: Less than 50% rusting
- E: More than 50% rusting

## (2) Foaming test

The evaluation was carried out according to a so-called Ross-clark method. 200 ml of a 1% aqueous solution of a sample was charged into a cylinder having an inner diameter of 50 mm and a height of 1000 mm while maintaining a sample temperature to  $20 \pm 1^\circ \text{C}$ . Air is continuously blown into the sample at a feed rate of 500 ml/min through a glass filter provided at the bottom of the cylinder and having a pore diameter of 40 to 50 microns. The height of the foam thus formed was measured after 60 seconds.

## (3) Cutting powder test

Five grams of dry cut wastage of cast iron (FC-20 and FC-25) was washed in hot toluene and, then, washed with methanol. The cutting wastage was dipped at an ambient temperature for 1 minute in an aqueous test sample solution containing 1% of the effective com-

ponent and having a pH of 9.5 (adjusted by sodium hydroxide). The cutting wastage was shaken free of the liquid and was placed on a filter paper in a Petri dish having a diameter of 60 mm. Then, 1 ml of the test sample solution was placed in the Petri dish. The Petri dish was covered and was allowed to stand under the conditions of a temperature of  $30 \pm 1^\circ \text{C}$ . and an R.H. of 80%. The rusting time and the rusting rating according to a JIS-K-2246 method after 24 hours were measured.

## (4) Dipping test

Dry cut wastage of cast iron (FC-25) was washed in the same manner as in the above cutting powder test and was, then, dipped in aqueous test sample solutions containing 0.5% and 1.0% of the effective component and having a pH of 9.5 (adjusted by sodium hydroxide). Thus, the period (in days) before which rusting occurred was measured.

## (5) Room exposure test

SPCC-1 steel test panels subjected to the same rust preventing treatment as in the above-mentioned evaluation test of rust preventing property under humidity conditions were allowed to stand at an ambient temperature in a room. The period in days before which rusting occurred was measured.

## (6) Match test

SPCC-1 steel and FC-20 cast iron test pieces were polished with No. 240 Emery paper and were washed with the solvents as in the above-mentioned cutting powder test. One drop of an aqueous test sample solution containing 0.25% of the effective component was placed on the surface of the test piece and, then, another test piece was laid thereover. The sandwich type assembly thus formed was allowed to stand for 24 hours under the conditions of a temperature of  $30 \pm 1^\circ \text{C}$ . and R.H. of 80%. The rusting of the sandwiched surfaces was visually observed.

○ . . . No rusting

△ . . . Partial rusting

× . . . More than 30% rusting

## (7) Non-ferrous metal corrosion test

Dipping corrosion test was carried out according to a JIS-K-2246 method. Test pieces were polished with no. 240 Emery paper and was washed in hot toluene and, then, washed with methanol. The test pieces were dipped in an aqueous test sample solution containing 1% of the effective component at a temperature of  $55 \pm 1^\circ \text{C}$ . for 7 days. The visual changes in the metal surface and the test sample solution were observed. The corrosion rate ( $\text{mg}/\text{cm}^2$ ) was obtained by determining the loss in weight before and after the dipping.

## (8) Salt water spray test

This test was carried out according to JIS-K-2246 and JIS-Z-2371 methods. The test sample treated in the same manner as in the above-mentioned test method 1) was sprayed with a 5% aqueous sodium chloride solution at  $35^\circ \text{C}$ . for the predetermined time by means of the specified salt water spray apparatus. The rusting degree was determined as follows.

A . . . No rusting

B . . . Less than 10% rusting

C . . . Less than 25% rusting

D . . . Less than 50% rusting

E . . . More than 50% rusting

TABLE 1

| Item<br>Condition<br>Sample | Humidity Test |    |    |    |    |    |    | Foaming<br>Test<br>mm | Cutting Powder Test  |         |                      |         | Dipping<br>Test<br>Rusting<br>Days | Room<br>Expo-<br>sure Test<br>Rusting<br>Days |     |     |
|-----------------------------|---------------|----|----|----|----|----|----|-----------------------|----------------------|---------|----------------------|---------|------------------------------------|-----------------------------------------------|-----|-----|
|                             | 5 hr          |    |    |    |    |    |    |                       | FC-20                |         | FC-25                |         |                                    |                                               |     |     |
|                             | Later         | 10 | 15 | 20 | 25 | 30 | 35 | 40                    | Rusting<br>Time (Hr) | Rusting | Rusting<br>Time (Hr) | Rusting |                                    |                                               |     |     |
| Example 1                   | A             | A  | A  | A  | A  | B  | B  | B                     | 5                    | >24     | A                    | >24     | A                                  | >20                                           | >20 | >30 |
| Example 2                   | A             | A  | A  | A  | A  | A  | A  | A                     | 5                    | >24     | A                    | >24     | A                                  | >20                                           | >20 | >30 |
| Example 3                   | A             | A  | A  | A  | A  | A  | A  | B                     | 5                    | >24     | A                    | >24     | A                                  | >20                                           | >20 | >30 |
| Comparative                 |               |    |    |    |    |    |    |                       |                      |         |                      |         |                                    |                                               |     |     |
| Example 1                   | A             | B  | E  | E  | —  | —  | —  | —                     | 5                    | 0.5     | E                    | 0.5     | E                                  | 3                                             | 15  | 10  |
| Comparative                 |               |    |    |    |    |    |    |                       |                      |         |                      |         |                                    |                                               |     |     |
| Example 2                   | A             | A  | B  | B  | C  | D  | E  | —                     | 250                  | 0.2     | E                    | 0.2     | E                                  | 2                                             | 10  | 7   |
| Comparative                 |               |    |    |    |    |    |    |                       |                      |         |                      |         |                                    |                                               |     |     |
| Example 3                   | A             | A  | A  | A  | A  | B  | B  | B                     | 5                    | 0.5     | D                    | 0.5     | C                                  | 3                                             | >20 | 14  |
| Comparative                 |               |    |    |    |    |    |    |                       |                      |         |                      |         |                                    |                                               |     |     |
| Example 4                   | A             | B  | E  | E  | —  | —  | —  | —                     | 110                  | 0.2     | E                    | 0.2     | E                                  | 2                                             | 12  | 7   |
| Comparative                 |               |    |    |    |    |    |    |                       |                      |         |                      |         |                                    |                                               |     |     |
| Example 5                   | A             | A  | A  | B  | B  | C  | D  | E                     | 180                  | 0.2     | E                    | 0.2     | D                                  | 3                                             | 15  | >30 |

TABLE 2

| Item<br>Condition<br>Sample | Match Test   |       |              |       |                  |                         | Non-ferrous Corrosion Test |                                |                       |                        |                                    |                         |                        |                  |                       |                        |  |
|-----------------------------|--------------|-------|--------------|-------|------------------|-------------------------|----------------------------|--------------------------------|-----------------------|------------------------|------------------------------------|-------------------------|------------------------|------------------|-----------------------|------------------------|--|
|                             | Cast<br>iron |       | Steel        |       | Copper           |                         | Zinc                       |                                | Brass                 |                        |                                    | Aluminum                |                        |                  |                       |                        |  |
|                             | Cast<br>iron | Steel | Cast<br>iron | Steel | Metal<br>surface | Liquid<br>observation   | Corro-<br>sion<br>rate     | Metal<br>surface               | Liquid<br>observation | Corro-<br>sion<br>rate | Metal<br>surface                   | Liquid<br>observation   | Corro-<br>sion<br>rate | Metal<br>surface | Liquid<br>observation | Corro-<br>sion<br>rate |  |
| Example 1                   | Δ            | o     | Δ            | —     | No<br>change     | Slight-<br>ly<br>bluish | -0.113                     | Partially<br>slight<br>greyish | No<br>change          | -0.094                 | Partially<br>slight<br>discoloring | Slight-<br>ly<br>bluish | -0.101                 | No<br>change     | No<br>change          | -0.004                 |  |
| Example 2                   | Δ            | o     | Δ            | —     | No<br>change     | Slight-<br>ly<br>bluish | -0.103                     | Partially<br>slight<br>greyish | No<br>change          | -0.099                 | Partially<br>slight<br>discoloring | Slight-<br>ly<br>bluish | -0.103                 | No<br>change     | No<br>change          | -0.003                 |  |
| Example 3                   | Δ            | o     | Δ            | —     | No<br>change     | Slight-<br>ly<br>bluish | -0.112                     | Partially<br>slight<br>greyish | No<br>change          | -0.085                 | Partially<br>slight<br>discoloring | Slight-<br>ly<br>bluish | -0.098                 | No<br>change     | No<br>change          | -0.004                 |  |
| Comparative                 | Δ            | Δ     | Δ            |       |                  |                         |                            |                                |                       |                        |                                    |                         |                        |                  |                       |                        |  |
| Example 1                   | x            | x     | x            |       |                  |                         |                            |                                |                       |                        |                                    |                         |                        |                  |                       |                        |  |
| Comparative                 | x            | Δ     | x            |       |                  |                         |                            |                                |                       |                        |                                    |                         |                        |                  |                       |                        |  |
| Example 2                   | x            | Δ     | x            |       |                  |                         |                            |                                |                       |                        |                                    |                         |                        |                  |                       |                        |  |
| Comparative                 | x            | x     | x            |       |                  |                         |                            |                                |                       |                        |                                    |                         |                        |                  |                       |                        |  |
| Example 3                   | x            | x     | x            |       |                  |                         |                            |                                |                       |                        |                                    |                         |                        |                  |                       |                        |  |
| Comparative                 | x            | x     | x            |       |                  |                         |                            |                                |                       |                        |                                    |                         |                        |                  |                       |                        |  |
| Example 4                   | Δ            | o     | x            |       |                  |                         |                            |                                |                       |                        |                                    |                         |                        |                  |                       |                        |  |
| Comparative                 | x            | Δ     | x            |       |                  |                         |                            |                                |                       |                        |                                    |                         |                        |                  |                       |                        |  |
| Example 5                   | x            | Δ     | x            |       |                  |                         |                            |                                |                       |                        |                                    |                         |                        |                  |                       |                        |  |

TABLE 3

| Sample    | Item<br>Kind of salt | Humidity Test |    |    |    |    |    |    | Foaming<br>Test<br>mm |
|-----------|----------------------|---------------|----|----|----|----|----|----|-----------------------|
|           |                      | 5 Hr<br>Later | 10 | 15 | 20 | 25 | 30 | 35 |                       |
| Example 3 | Na                   | A             | A  | A  | A  | A  | B  | B  | 5                     |
| "         | K                    | A             | A  | A  | A  | A  | B  | B  | 5                     |
| "         | NH <sub>4</sub>      | A             | A  | A  | A  | B  | B  | C  | 5                     |
| "         | Methylamine          | A             | A  | A  | A  | A  | B  | B  | 5                     |
| "         | Monoethanolamine     | A             | A  | A  | A  | A  | B  | B  | 6                     |
| "         | Diethanolamine       | A             | A  | A  | A  | A  | A  | B  | 5                     |
| "         | Cyclohexylamine      | A             | A  | A  | A  | A  | B  | B  | 5                     |

TABLE 3-continued

| Sample    | Item<br>Kind of salt | Humidity Test |    |    |    |    |    |    | Foaming<br>Test<br>mm |
|-----------|----------------------|---------------|----|----|----|----|----|----|-----------------------|
|           |                      | 5 Hr<br>Later | 10 | 15 | 20 | 25 | 30 | 35 |                       |
| "         | Morpholine           | A             | A  | A  | A  | A  | B  | B  | 6                     |
| Example 4 | Triethanolamine      | A             | A  | A  | B  | B  | B  | C  | .5                    |
| Example 5 | "                    | A             | B  | E  | E  | —  | —  | —  | 6                     |
| Example 6 | "                    | A             | A  | B  | B  | C  | E  | E  | 5                     |

TABLE 4

| Sample      | Kind of Salt | Humidity Test |        |          |        | Salt Water Spray Test |       |        |          |       |        |
|-------------|--------------|---------------|--------|----------|--------|-----------------------|-------|--------|----------|-------|--------|
|             |              | Spindle oil   |        | Kerosine |        | Spindle oil           |       |        | Kerosine |       |        |
|             |              | 15 Day        | 30 Day | 15 Day   | 30 Day | 3 Hr                  | 6 Day | 24 Day | 3 Day    | 6 Day | 24 Day |
| Example 7   | Ca           | A             | A      | A        | A      | A                     | A     | B      | A        | A     | B      |
| "           | Mg           | A             | A      | A        | A      | A                     | B     | E      | A        | B     | E      |
| "           | Ba           | A             | A      | A        | A      | A                     | A     | B      | A        | A     | B      |
| No addition | —            | C             | E      | C        | E      | E                     | E     | E      | E        | E     | E      |

## EXAMPLE 8

Forty three parts of aminocaproic acid, 25 parts of sodium hydroxide and 140 parts of water were charged into a reaction vessel provided with a condenser and a stirrer. The mixture was stirred and a solution of 30 parts of terephthaloyl chloride dissolved in 70 parts of dioxane was dropwise added thereto while cooling so as to maintain the temperature of the reaction mixture at 30° C. or less. After the completion of the dropwise addition, the reaction mixture was stirred for 3 hours at a temperature of 30° C. and, then, was neutralized with sulfuric acid while cooling.

The white precipitate thus formed was filtered and was washed with water. Then, the precipitate was purified in isopropyl alcohol to obtain N,N'-terephthaloyl diaminocaproic acid.

Thirty parts of N,N'-terephthaloyl diaminocaproic acid obtained above was mixed with 26 parts of triethanolamine and 132 parts of water under heating to prepare a rust preventing composition containing about 30% of the effective component.

## EXAMPLE 9

Fifteen parts of N,N'-terephthaloyl diaminocaproic acid obtained in Example 8 was mixed with 3 parts of sodium hydroxide and 42 parts of water under heating to prepare a rust preventing composition containing about 30% of the effective component.

## EXAMPLE 10

Fifteen parts of N,N'-terephthaloyl diaminocaproic acid obtained in Example 8 was mixed with 4.5 parts of potassium hydroxide and 45.5 parts of water under heating to prepare a rust preventing composition containing about 30% of the effective component.

## EXAMPLE 11

Fifteen parts of N,N'-terephthaloyl diaminocaproic acid obtained in Example 8 was mixed with 8 parts of diethanolamine and 54 parts of water under heating to prepare a rust preventing composition containing about 30% of the effective component.

## EXAMPLE 12

Fifteen parts of N,N'-terephthaloyl diaminocaproic acid obtained in Example 8 was mixed with 4 parts of methylamine and 44 parts of water under heating to

30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7

and, then, was neutralized with sulfuric acid to precipitate the resultant dicarboxylic acid.

The dicarboxylic acid was filtered and washed with water. Thus, N,N'-phthaloylbis(DL-alanine) in the form of white powder was obtained.

Thirty parts of N,N'-phthaloylbis(DL-alanine) was mixed with 45 parts of triethanolamine and 175 parts water to prepare a rust preventing composition containing about 30% of the effective component.

#### Comparative Example 6

5

One hundred parts of benzoic acid, 117 parts of triethanolamine and 506 parts of water were mixed under heating while stirring to obtain a rust preventing composition containing about 30% of the effective component.

10

#### Comparative Example 7

One hundred parts of oleic acid, 51 parts of triethanolamine and 352 parts of water were mixed under heating while stirring to obtain a rust preventing composition containing about 30% of the effective component.

The rust preventing compositions prepared in Examples 8 to 16 and Comparative Examples 6 and 7 were evaluated. The results are shown in Tables 5 and 6. Table 5 shows the results of the rusting test according to a JIS-K-2246 method mentioned above and the foaming test mentioned above. Table 6 shows the results of the rusting test according to a JIS-K-2246 method mentioned above, in which correlations between the rusting time and the rusting rating are shown.

TABLE 5

| Sample      | Rusting Rating |          |          |          |          |          |          |          | Foaming (mm) |
|-------------|----------------|----------|----------|----------|----------|----------|----------|----------|--------------|
|             | 5 Hr Later     | 10 Later | 15 Later | 20 Later | 25 Later | 30 Later | 35 Later | 40 Later |              |
| Example 8   | A              | A        | A        | A        | A        | A        | A        | A        | 5            |
| Example 9   | A              | A        | A        | A        | A        | A        | B        | B        | 6            |
| Example 10  | A              | A        | A        | A        | A        | A        | B        | B        | 5            |
| Example 11  | A              | A        | A        | A        | B        | B        | C        | C        | 5            |
| Example 12  | A              | A        | A        | A        | A        | B        | B        | C        | 5            |
| Example 13  | A              | A        | A        | A        | A        | B        | B        | C        | 6            |
| Example 14  | A              | A        | A        | A        | A        | B        | B        | C        | 6            |
| Example 15  | A              | A        | A        | A        | A        | A        | A        | B        | 5            |
| Example 16  | A              | A        | A        | A        | A        | B        | B        | B        | 5            |
| Comparative | A              | B        | B        | E        | E        | E        | E        | E        | 7            |
| Example 6   |                |          |          |          |          |          |          |          |              |
| Comparative | A              | A        | B        | C        | D        | D        | E        | E        | 250          |
| Example 7   |                |          |          |          |          |          |          |          |              |

TABLE 6

| Sample      | FC-20            |                | FC-25            |                | 55 |
|-------------|------------------|----------------|------------------|----------------|----|
|             | Rusting Time (H) | Rusting Rating | Rusting Time (H) | Rusting Rating |    |
| Example 8   | >24              | A              | >24              | A              |    |
| Example 9   | 20               | B              | >24              | A              |    |
| Example 10  | 20               | B              | 20               | B              |    |
| Example 11  | 20               | B              | >24              | A              |    |
| Example 12  | 15               | C              | 20               | B              |    |
| Example 13  | >24              | A              | >24              | A              |    |
| Example 14  | >24              | A              | >24              | A              |    |
| Example 15  | 20               | B              | 20               | B              |    |
| Example 16  | >24              | A              | >24              | A              |    |
| Comparative | 0.5              | E              | 0.5              | E              |    |
| Example 6   |                  |                |                  |                |    |
| Comparative | 0.5              | E              | 0.5              | E              |    |
| Example 7   |                  |                |                  |                |    |

The results shown in Tables 1 to 6 clearly indicate the following advantages of the present invention.

- (1) The rust inhibitors of the present invention exhibited excellent rust preventing properties equal to, or superior to, those of the known rust inhibitors having an excellent rust preventing property and the rust preventing composition containing a known typical rust preventing compound, sodium nitrite.
- (2) The rust inhibitors of the present invention have a poor foaming property, in addition to excellent rust preventing properties, and, therefore, are readily applicable to metals without causing a decrease in the rust preventing properties caused by foaming.
- (3) The rust inhibitors of the present invention exhibited excellent rust preventing properties and effects all in the humidity test, the cutting powder test, the dipping test, the room exposure test, the match test and the salt water spray test. Contrary to this, the comparative rust inhibitors did not necessarily exhibit good results in all the above-mentioned tests. This means that the rust inhibitors of the present invention can be usefully applied to any substrates used under various conditions.
- (4) The rust inhibitors of the present invention exhibited excellent rust preventing properties, even without using inorganic salt type rust inhibitors such as sodium nitrite, as different from conventional organic type rust inhibitors.
- (5) The rust inhibitors of the present invention have excellent rust preventing properties not depending upon the kinds of the compounds, although some changes in the rust preventing properties were observed.

(6) The water-soluble type rust inhibitors of the present invention can be readily removed from the substrates by washing with water. Thus, the post-treatment is easy and there is no adverse effect in the post-treatment step.

(7) The rust inhibitors of the present invention caused no substantial or little corrosion against non-ferrous metals. Thus, no substantial corrosion problem occurs when the rust inhibitor of the present invention is applied to non-ferrous metals. The results similar to those shown in Table 2 were obtained in the other non-ferrous metals. Especially when the present rust inhibitors in the form of sodium salt were used, no corrosion on the metal surfaces and no visual changes in the test solutions were observed. It should be noted, however, that the combined use of another type of rust inhibitor or agents together with the present rust inhibitors

may be advantageous to effect a perfect corrosion resistance of non-ferrous metals.

(8) The present rust inhibitors in the form of polyvalent metal salts were oil-soluble type rust preventing components and exhibited good rust preventing properties even in the case of the humidity test and the salt water spray test.

We claim:

1. A method for inhibiting rust on a metal which comprises:

treating the metal with a rust inhibitor comprising, as an effective component, at least one compound having the following general formulae (A), (B), and (C)



and



wherein R<sub>1</sub> and R<sub>2</sub> are independently a hydrocarbon group having 1 to 6 carbon atoms, R<sub>3</sub> and R<sub>4</sub> are independently a hydrocarbon group having 1 to 4 carbon atoms or a hydrocarbon group containing an aromatic ring and having 6 to 12 carbon atoms, R<sub>5</sub> and R<sub>6</sub> are

independently a hydrocarbon group having 1 to 18 carbon atoms, m and n are independently 0 or an integer of 1 to 3, R<sub>3</sub> or R<sub>4</sub> being hydrogen in the case of m or n being 0, X is O, S, SO<sub>2</sub>, CO or a hydrocarbon having 1 to 9 carbon atoms, Y is an aromatic hydrocarbon group having 6 to 10 carbon atoms and M is a cation, said rust inhibitor being in the form of a solution, a dispersion, or an emulsion.

2. A method as claimed in claim 1, wherein said compound has the general formula (A).

3. A method as claimed in claim 2, wherein R<sub>1</sub> and R<sub>2</sub> are independently a hydrocarbon group having 1 to 3 carbon atoms in the general formula (A).

4. A method as claimed in claim 2, wherein R<sub>3</sub> and R<sub>4</sub> are independently hydrogen or a methyl group in the general formula (A).

5. A method as claimed in claim 2, wherein X is O, SO<sub>2</sub>, or a hydrocarbon group having 1 to 4 carbon atoms in the general formula (A).

20 6. A rust inhibitor as claimed in claim 1, wherein said compound has the general formula (B).

7. A rust inhibitor as claimed in claim 1, wherein said compound has the general formula (C).

25 8. A method as claimed in claim 1, wherein said compound has the general formula (A) wherein R<sub>1</sub> and R<sub>2</sub> are independently a hydrocarbon group having 1 to 3 carbon atoms, R<sub>3</sub> and R<sub>4</sub> are hydrogen or a methyl group, and X is O, SO<sub>2</sub>, or a hydrocarbon group having 1 to 4 carbon atoms.

30 9. A rust inhibitor as claimed in claim 1, wherein said compound has the general formula (B) wherein R<sub>1</sub> and R<sub>2</sub> are independently a hydrocarbon group having 1 to 3 carbon atoms, R<sub>3</sub> and R<sub>4</sub> are hydrogen or a methyl group, and X is O, SO<sub>2</sub>, or a hydrocarbon group having 1 to 4 carbon atoms.

\* \* \* \* \*

40

45

50

55

60

65